

[54] NON-POISONOUS ZINC PLATING BATHS

[76] Inventors: Hidenori Hayashida, 210 Higashi Amakawa-cho, Takatsuki; Ryoji Nakahara, 440 Deguchi, Hirakata, both of Japan

[22] Filed: Apr. 7, 1971

[21] Appl. No.: 132,218

## [30] Foreign Application Priority Data

Apr. 24, 1970 Japan..... 45-34717

[52] U.S. Cl. .... 204/55 R, 204/DIG. 2

[51] Int. Cl. .... C23b 5/12, C23b 5/46

[58] Field of Search..... 204/55, DIG. 2

## [56] References Cited

## UNITED STATES PATENTS

|           |         |                    |          |
|-----------|---------|--------------------|----------|
| 2,813,065 | 11/1957 | Du Rose .....      | 204/45   |
| 3,296,104 | 1/1967  | Eppensteiner ..... | 204/55 R |
| 3,296,105 | 1/1967  | Rushmere .....     | 204/55 R |
| 3,594,291 | 7/1971  | Todt et al. ....   | 204/55 R |
| 2,389,179 | 11/1945 | Brown.....         | 204/49   |
| 2,389,181 | 11/1945 | Brown.....         | 204/49   |
| 3,655,534 | 4/1972  | Kampe.....         | 204/55   |

Primary Examiner—F. C. Edmundson  
Attorney, Agent, or Firm—Hammond and Littell

## [57] ABSTRACT

A non-poisonous zinc plating bath comprising a fundamental plating composition including zinc salt and ammonium salt with or without hydroxy carboxylic acid; a sulfate compound or compounds having the general formula A—B—(CH<sub>2</sub>CH<sub>2</sub>O)<sub>2-100</sub>SO<sub>3</sub>M; an alkynaphthylketon compound or compounds having the general formula



and a nitrogen-containing heterocyclic ring compound or compounds substituted with carboxyl group having the general formula



or mixture thereof.

5 Claims, No Drawings

## NON-POISONOUS ZINC PLATING BATHS

## BACKGROUND OF THE INVENTION

This invention relates to novel and improved non-poisonous zinc plating baths which contain no cyanide therein and which can effectively eliminate occurrence of harmful environmental contamination even when the waste liquids from the baths are discarded out of the system.

One typical prior art zinc plating bath for use in zinc-plating the surfaces of various base metals has the composition which principally comprises 80 g/l of sodium hydroxide, 35 g/l of  $Zn^{2+}$  and 100 g/l of sodium cyanide and the waste liquid from the plating bath includes cyan-containing substances in a substantially high concentration. Therefore, when the waste liquid is discarded out of the system into a river or sea, for example, the liquid will seriously contaminate the water in the river or sea.

Of late, low cyan-concentration zinc plating baths containing  $Zn^{2+}$  and sodium cyanide in relatively lower concentrations have been proposed and practically employed. These plating baths generally contain as their principal components 80 g/l of sodium hydroxide, 8 g/l of  $Zn^{2+}$  and 10 g/l of sodium cyanide and in fact, these plating baths, contain sodium cyanide in a lower concentration than the prior art zinc plating baths do.

However, since these recently developed zinc plating baths still contain sodium cyanide therein though the concentration of the cyanide is substantially lower than that of the corresponding component in the comparative prior art zinc plating baths, it is, of course, evident that the low cyan-containing zinc plating baths will still inevitably contaminate the water in a river or sea when the waste liquid from these baths is discarded there. And since the concentration of sodium cyanide in these baths is substantially low, the brilliance-imparting current density range available in these plating baths is limited and current efficiency in these baths is also low to the degree that the productivity of these baths will be substantially reduced.

In order to eliminate the difficulties referred to just above, there has been, of quite late, proposed and partially employed a brilliant zinc plating bath which contains no cyanide therein and the brilliant zinc plating bath is disclosed in French Pat. No. 1,524,719. However, it has been found that the brilliant zinc plating bath of the above-mentioned French Patent is still not perfectly satisfactory and especially, is not satisfactory with respect to the brilliance-imparting current density range available.

## SUMMARY OF THE INVENTION

Therefore, one principal object of the present invention is to provide a non-poisonous zinc plating bath which contains no cyanide therein and which can effectively eliminate the disadvantages inherent in the conventional zinc plating baths which contain cyanide in varying concentrations or contain no cyanide therein.

Another object of the present invention is to provide a non-poisonous zinc plating bath which contains no cyanide therein whereby even when the waste liquid from the bath is discarded out of the system to the environment, there will be no harmful environmental contamination to occur.

Another object of the present invention is to provide a non-poisonous zinc plating bath which has a wide range of brilliance-imparting current density available, can be effectively applicable to barrel plating, is excellent in performance and will not cause harmful environmental contamination.

Basically, the non-poisonous zinc plating bath of the present invention generally comprises (a) a conventional zinc plating composition comprising zinc salts and ammonium salt with or without hydroxy carboxylic acid; (b) a sulfate compound or compounds of polyether having the below-mentioned general formula:



15

wherein A is hydrogen,  $CnH_{2n+1}$  ( $n$  is an integral within the range of 4 - 20), alkylphenylene, residue after removal of the hydroxy group from molecules of 20 sorbitol or mannitol or residue of alkylpolyamine, B is a bridge selected from the group comprising  $-COO-$ ,  $-NH-$ ,  $-S-$ ,  $-O-$ ,  $-(OCH_2CH_2CH_2O)_{2+30}$  and  $-CONH-$  and M is hydrogen, ammonium or a metal selected from the group comprising, sodium, potassium, magnesium, calcium and zinc; (c) an alkyl-naphthylketon compound or compounds having the below-mentioned general formula:



(2)

wherein  $R_1$  is a group selected from the group comprising alkyl, phenyl, methylnaphthyl, styryl, nitrophenylene and aminophenylene and  $R_2$  is a group selected from the group comprising hydrogen, halogen, alkyl, aryl, sulfo, amino, nitro, hydroxyl, carboxyl and formyl; and (d) a nitrogen-containing heterocyclic ring compound or compounds substituted with carboxyl group having the below-mentioned general formula:



(3)

45 wherein



50 is a heterocyclic ring selected from the group comprising pyridine, quinoline and isoquinoline and R is a group selected from the group comprising hydrogen, halogen, alkyl, alkoxy, aryl, amino, nitro, hydroxyl, carboxyl, sulfo, sulfomoyl, substituted sulfomoyl, hydroxycarboxyalkyl, carboxy vinylene, carboxy phenylene, carboxyalkyl phenylvinylene and mercapto.

## EXAMPLES OF THE INVENTION

60 Zinc salts, ammonium salts and hydroxy carboxylic acids to be blended with the other components of the zinc plating baths of the invention may be those usually employed in the conventional zinc plating baths compositions and the zinc salts useful in the baths of the invention include zinc chloride, zinc sulfate and zinc sulfamate. These zinc salts can be employed in amounts ranging from 10 to 200 g/l. The ammonium salts useful

in the baths of the invention include ammonium chloride, ammonium sulfate and ammonium acetate and these ammonium salts can be employed in amounts ranging from 20 to 350 g/l with satisfactory results. The hydroxy carboxylic acids useful in the baths of the invention include maleic acid, citric acid, gluconic acid, tartaic acid and lactic acid and these hydroxy carboxylic acids can be optionally employed in amounts ranging from 1 to 100 g/l.

In preparing the zinc plating baths of the invention, any one of the above-mentioned zinc salts and any one of the above-mentioned ammonium salts are blended together or alternatively, anyone of the above-mentioned hydroxy carboxylic acids is further added to the blend. Thereafter, the resulting mixture is added thereto the compounds represented by the general formulas (1), (2) and (3), respectively, thereto to prepare non-poisonous zinc plating baths. In order to simplify the disclosure herein and also for better understanding of the invention, the mixture of zinc and ammonium salts with or without hydroxy carboxylic acid will be referred to as the "fundamental bath composition" hereinafter.

The operative effects of the additive organic compounds represented by the general formulas (1), (2) and (3), respectively when they are added to the fundamental bath composition to prepare a zinc plating bath will be described hereinbelow.

Firstly, the nitrogen-containing heterocyclic ring compound or compounds substituted with carboxyl group having the general formula (3) have buffering action upon the pH of the plating bath thereby to facilitate the pH control of the plating bath.

Secondly, the nitrogen-containing heterocyclic ring carboxylic acid compound or compounds extend the current density range of the plating bath available to impart brilliance to the surfaces of a base metal to be plated and in other words, the compound or compounds serve to reduce the necessary brilliance-imparting currency density from a higher value portion thereby to substantially improve the brilliance and covering power of deposit metal on the base metal even when the bath is employed for barrel plating which must be usually carried out at a relatively low current density. An example for manifesting the improvements with respect to both the brilliance and covering power of deposit metal obtainable by the plating bath of the invention with the addition of the nitrogen-containing heterocyclic ring compound or compounds over those obtainable by a control zinc plating bath without the addition of such a compound will be given hereinbelow. When a zinc plating bath comprising 120 g/l of zinc chloride, 180 g/l of ammonium chloride, 20 g/l of sodium gluconate, 0.5 g/l of 2-ethylnaphthylketon and 10 g/l of  $C_9H_{16}O-(CH_2CH_2)_{20}SO_3Na$  was employed for zinc-plating a base metal, it was found that the available brilliance-importing current density range stood in a rather high region such as being 16-20 A/dm<sup>2</sup> and the available range was very limited one as seen from the value shown above.

Such a zinc plating bath cannot be employed for rack and barrel platings which require the brilliance-imparting current density range of 0.5-20 A/dm<sup>2</sup> and 0.1-3 A/dm<sup>2</sup>, respectively. However, when the above-mentioned control bath was added thereto 3 g/l of quinaldic acid which is a typical nitrogen-containing heterocyclic ring compound substituted

base metal, it was surprisingly found that the brilliance-imparting current density range of the bath containing the carboxylic acid compound was extended to the range of 0.1 - 20 A/dm<sup>2</sup> and could be suitably employed for plating articles having complicate contours and shapes with satisfactory results. It was also found that the bath with the addition of the carboxylic acid compound could be satisfactorily employed for barrel plating which would generally require a relatively low current density. Now, description will be made of the suitable amount range of a nitrogen-containing heterocyclic ring compound substituted with carboxyl group having such effects to be added to the fundamental bath composition according to the teach of the present invention. When one or more of the above-mentioned heterocyclic ring compound substituted with carboxyl group are employed in amounts less than 0.1 g/l in the bath, the additive acid compound or compounds cannot be expected to exhibit the above-mentioned effects and on the other hand, when the acid compound or compounds are employed in amounts greater than 15 g/l, although the brilliance and covering power of deposit metal obtainable at a relatively low current density will not be adversely affected in any way, there is the tendency to render the deposit metal layer brittle. Thus, the amount range of the additive carboxylic acid compound or compounds is preferably within the range of 0.1 - 15 g/l. And the pH of the zinc plating bath of the invention is preferably maintained within the range of 3.0 - 10. The reason is that when the pH is below 3.0, the plated product will be readily subjected to corrosion and the additive carboxylic acid compound or compounds will salt out and on the other hand, when the pH is over 10, the ammonia contained in the bath is allowed to disperse by evaporation. Therefore, the pH of the bath is preferably maintained within the range of 3 - 10.

The temperature of the plating bath is preferably maintained within the range of 10°-50°C. Although plating operations employing baths of the non-poisonous zinc plating compositions of the invention can be performed while the baths being maintained static, better results will be obtained when the baths are air-agitated or by the adoption of the so-called cathode rocker system. Typical nitrogen-containing heterocyclic ring compounds substituted with carboxyl group which are suitably employed in the present invention will be given hereinbelow, and in connection with this it is to be understood that they can be employed either in their simple forms or in the forms of various mixtures thereof.

1. 2-methyl-3-carboxy pyridine
2. 5-acetyl-3-carboxy pyridine
3. 2-hydroxy-4-carboxy-6-acetyl pyridine
4. 2-methoxy-3-carboxy pyridine
5. 3-nitro-4-carboxy pyridine
6. 2-amino-4-carboxy pyridine
7. 2-sulfo-4-Carboxy pyridine
8. nicotinic acid
9. 6-chloro-4-carboxy pyridine
10. quinaldic acid
11. 4-carboxy isoquinoline
12. 5-carboxy-8-hydroxy quinoline
13. 7-amino-3-carboxy quinoline
14. 7-acetyl-3-carboxy quinoline
15. 5-mercaptop-3-carboxy quinoline

Next, description will be made of the operative effects the additive sulfate compounds of polyether having the general formula (1) referred to above and to be added to the fundamental bath composition of the baths of the invention. Firstly, the sulfate compound or compounds of polyether accelerate the dissolution of alkynaphthylketon compound or compounds having the general formula (2) referred to above and to be also added to the fundamental bath composition of the invention into the baths. This action of the sulfate compound or compounds will be further accelerated by selecting ester of sulfuric acid as the end group of the polyether compound or compounds to be employed in the present invention. Furthermore, such an action of the sulfate compound or compounds of polyether serves to increase the salting-out temperature and to facilitate the control of the plating baths.

Secondly, the sulfate compound or compounds of polyether when employed in conjunction with the fundamental bath composition serve to suitably control the electrodeposition of zinc and this is considered due to the fact that a thin colloidal film is probably formed in the cathode because of the structure of  $-\text{CH}_2\text{CH}_2\text{O}-$  present in the molecules of the polyether compound or compounds.

Thirdly, the sulfate compound or compounds of polyether may serve to control extra-ordinary deposition of zinc at high current densities thereby to prevent the formation of dendrite.

As to the suitable amount of the sulfate compound or compounds of polyether to be added to the baths of the invention, when the sulfate compound or compounds are employed in amounts less than 0.1 g/l, the above-mentioned operative effects cannot be fully realized and on the other hand, when the amount is over 30 g/l, the obtained deposit metal will be brittle and will be readily subjected to salting-out. Therefore, the sulfate compound or compounds of polyether are preferably employed in amounts from 0.1 to 30 g/l.

Typical sulfate compounds of polyether to be employed in the baths of the present invention will be shown hereinbelow by their chemical formulas. These sulfate compounds may be employed either in their simple forms or in the forms of mixtures thereof with the same plating performances,

1.  $\text{C}_9\text{H}_{19}-\text{COO}-\text{CH}_2\text{CH}_2\text{O}-\text{SO}_3\text{Na}$
2.  $\text{C}_8\text{H}_{17}-\text{NH}-\text{CH}_2\text{CH}_2\text{O}-\text{SO}_3\text{Na}$
3.  $\text{HS}-\text{CH}_2\text{CH}_2\text{O}-\text{SO}_3\text{Na}$
4.  $\text{C}_9\text{H}_{19}-\text{C}_6\text{H}_4-\text{O}-\text{CH}_2\text{CH}_2\text{O}-\text{SO}_3\text{Na}$
5.  $\text{C}_8\text{H}_{17}-\text{S}-\text{CH}_2\text{CH}_2\text{O}-\text{SO}_3\text{Na}$
6.  $\text{C}_6\text{H}_{13}-\text{COO}-\text{CH}_2\text{CH}_2\text{O}-\text{SO}_3\text{Na}$
7.  $\text{C}_7\text{H}_{15}-\text{COHN}-\text{CH}_2\text{CH}_2\text{O}-\text{SO}_3\text{Na}$
8.  $\text{C}_{10}\text{H}_{21}-\text{C}_6\text{H}_4-\text{S}-\text{CH}_2\text{CH}_2\text{O}-\text{SO}_3\text{Na}$
9.  $\text{C}_4\text{H}_9-\text{NH}-\text{CH}_2\text{CH}_2\text{O}-\text{SO}_3\text{Na}$
10.  $\text{C}_9\text{H}_{19}-\text{C}_6\text{H}_4-\text{CONH}-\text{CH}_2\text{CH}_2\text{O}-\text{SO}_3\text{Na}$
11.  $\text{H}-\text{O}-\text{CH}_2\text{CH}_2\text{O}-\text{SO}_3\text{Na}$
12.  $\text{H}-\text{O}-\text{CH}_2\text{CH}_2\text{O}-\text{CH}_2\text{CH}_2\text{CH}_2\text{O}-\text{SO}_3\text{Na}$   
 $\quad +\text{CH}_2\text{CH}_2\text{O}-\text{SO}_3\text{Na}$

13.



Next, description will be made of the operative effects of the alkynaphthylketon compounds having the general formula (2) referred to above to be added to the zinc plating baths of the present invention. The alkynaphthylketon compound or compounds serve to impart brilliance to deposit metal in the plating baths. The addition of the compound or compounds having the general formula (2) is necessary because plating baths comprising the fundamental plating composition having only the sulfate compound or compounds of polyether of the general formula (1) and the nitrogen-containing heterocyclic ring compound or compounds substituted with carboxyl group of the general formula (3) cannot produce bright deposit metal and will produce semi-bright deposit metal at the best.

However, it has been found that when an alkynaphthylketon compound or compounds are added to the zinc plating bath comprising the above-mentioned fundamental composition having the compound or compounds of the general formula (1) and the compound or compounds of the general formula (3) added thereto, a surprising bright plating can be attained. For example, when a zinc plating bath was prepared by adding 0.8 g/l of an alkynaphthylketon compound to the fundamental composition having a sulfate compound of polyether in an amount in the range referred to above and a heterocyclic ring compound substituted with carboxyl group in an amount in the range referred to above added thereto it was possible to produce a bright plated product whose brilliance substantially corresponded to that of a bright nickel-plated product. The brilliance obtained by the use of the alkynaphthylketon compound as one of the three types of additives was confirmed as to be due to the presence of the naphthalene in the additive compound through the below-given comparison experiments. In some of the experiments, zinc plating baths were prepared by adding acetophenone in the amount range from 0.1 to 20 g/l to the fundamental composition including a sulfate compound or compounds of polyether in the above-mentioned amount range and a heterocyclic ring compound or compounds substituted with carboxyl group in the above-mentioned amount range as taught in the above-mentioned French patent, but the brilliance-imparting current density range of these baths was narrow such as being 0.5 - 2 A/dm<sup>2</sup> whereas in the others of the experiments, plating baths were prepared by adding an alkynaphthylketon compound or compounds in the above-mentioned amount range to the fundamental composition including the compound or compounds of the general formula (1) and the compound or compounds of the general formula (3) without the use of acetophenone and the brilliance-imparting current density of these baths was found

wider such as being 0.1 to 20 A/dm<sup>2</sup> and bright plated products were obtained over. As to the suitable amount of an alkynaphthylketon compound or compounds to be added to the plating baths of the invention, when the compound or compounds having the general formula (2) are employed in amounts less than 0.1 g/l, the brilliance-imparting effects of the baths are insufficient and on the other hand, when the compound or compounds of the general formula (2) are employed in amounts in excess of 5.0 g/l, the obtained deposit metal will be brittle. Therefore, the compound or compounds of the general formula (2) should be employed in the range from 0.01 to 5.0 g/l. Typical examples of alkynaphthylketon compounds usefully employed in the zinc plating baths of the invention are given hereinbelow and they can be employed either in their simple forms or in the forms of mixtures thereof without departing from the spirit and scope of the invention with the same results.

1. 5-chloro-2-acetonaphthone
2. 5-methyl-2-acetonaphthone
3. 5-amino-1-acetonaphthone
4. 1,5-diacetonaphthone
5. acetonaphthone (1 or 2)
6. 2-phenylnaphthylketone
7. 1,1'-dinaphthylketone
8. 1-styrylnaphthylketone
9. p-aminophenyl-1-naphthylketone
10. p-nitrophenyl-2-naphthone
11. 1-hydroxy-4-acetonaphthone

12. 1-hydroxy-4-chloro-2-acetonaphthone  
 13. 1-carboxy-5-acetonaphthone  
 14. 5-formyl-1-acetonaphthone  
 15. 3-amino-2-methoxy-1-acetonaphthone

5 In the foregoing, description has been made of the operative effects of the various additives to be employed in conjunction with the fundamental plating bath composition according to the present invention, but in order to manifest the excellent operative effects of the baths having the above-mentioned composition of the invention over those obtainable by the prior art zinc plating baths, the following comparison experiments were conducted using the baths of the invention and those of the prior art. In any of these experiments, 10 the fundamental composition comprised 90 g/l of zinc chloride, 180 g/l of ammonium chloride and 20 g/l of tartaric acid and the fundamental composition was added thereto the additives as shown in the below-given Table 1 (prior art) and Table 2 (the invention), 15 respectively to prepare the zinc plating baths. Test pieces were zinc-plated using the thus prepared baths under the conditions such as the temperature of 30°C, the current density of 3 A/dm<sup>2</sup> and pH of 5.0 while agitating the baths with air. The zinc-plated test pieces 20 were measured or observed in accordance with the Hull cell test procedure for the leveling and appearance of the plated products and the brilliance-imparting current density and of the baths. The results of these measurement or observation are given in the Table 1 and 25 Table 2, respectively.

30

Table 1

| No. | additive<br>or<br>additives                                                                                               | Results obtained by the use of prior art zinc plating baths |                                                         |                                                                                             |           | appearance                                                           |
|-----|---------------------------------------------------------------------------------------------------------------------------|-------------------------------------------------------------|---------------------------------------------------------|---------------------------------------------------------------------------------------------|-----------|----------------------------------------------------------------------|
|     |                                                                                                                           | throwing<br>power<br>(g/l)                                  | Brill-<br>iance in-<br>dex of<br>reflec-<br>tion<br>(%) | brilli-<br>ance-<br>impart-<br>ing cu-<br>rrent<br>density<br>range<br>(A/dm <sup>2</sup> ) |           |                                                                      |
| 1   | None                                                                                                                      | 0                                                           | 43                                                      | 3                                                                                           | —         | lustreless<br>rough dendrite<br>lustreless                           |
| 2   | C <sub>6</sub> H <sub>4</sub> (OH)COONa                                                                                   | 2                                                           | 45                                                      | — 5                                                                                         | —         | Lustreless<br>no rough dendrite in high<br>current density<br>region |
| 3   | C <sub>6</sub> H <sub>4</sub> (COONa) <sub>2</sub>                                                                        | 2                                                           | 41                                                      | 7                                                                                           | —         | light amber<br>color brilliancy<br>in low current<br>density portion |
| 4   | C <sub>6</sub> H <sub>17</sub> —C <sub>6</sub> H <sub>4</sub> —O—<br>—(CH <sub>2</sub> CH <sub>2</sub> O) <sub>30</sub> H | 10                                                          | 44                                                      | 15                                                                                          | 0.5 – 2.0 | ditto                                                                |
| 5   | C <sub>6</sub> H <sub>5</sub> OCH <sub>3</sub> CHO                                                                        | 2                                                           | 45                                                      | 17                                                                                          | 0.5 – 2.0 | —                                                                    |
|     | C <sub>6</sub> H <sub>19</sub> —C <sub>6</sub> H <sub>4</sub> —O—<br>—(CH <sub>2</sub> CH <sub>2</sub> O) <sub>30</sub> H | 10                                                          |                                                         |                                                                                             |           |                                                                      |
|     | C <sub>6</sub> H <sub>5</sub> COOH                                                                                        | 2                                                           |                                                         |                                                                                             |           |                                                                      |
|     | C <sub>6</sub> H <sub>19</sub> —C <sub>6</sub> H <sub>4</sub> —O—<br>—(CH <sub>2</sub> CH <sub>2</sub> O) <sub>30</sub> H | 10                                                          |                                                         |                                                                                             |           |                                                                      |

<sup>1</sup>The values of the throwing power given in the above Table were obtained in accordance with the Haring H.E. and Blum W Procedure [Trans. Am. Electrochem. Soc. 313 (1923)].

<sup>2</sup>The values of the brilliance (index of reflection) given in the above Table were obtained by the use of a precision photoelectric color meter produced by the Tokyo Shibaura Electric K.K. of Tokyo.

<sup>3</sup>The appearance of the processed test pieces were observed after 5 minutes of immersion thereof in the baths with the total current of 3 amperes.

TABLE 2

(Results obtained by the use of the zinc plating baths of the invention)

| Number | Additives (g./l.)                                        | Throwing power, percent | Brilliance (index of reflection) percent | Brilliance (imparting current density range) A./dm. <sup>2</sup> | Appearance                              |
|--------|----------------------------------------------------------|-------------------------|------------------------------------------|------------------------------------------------------------------|-----------------------------------------|
| 1..... | $C_9H_{19}-O-(CH_2CH_2O)_{15}-SO_3Na$                    | 10                      |                                          |                                                                  |                                         |
|        |                                                          | 2                       |                                          |                                                                  |                                         |
|        |                                                          | 1                       | 44                                       | 88                                                               | 0.2-20 Brilliance on the whole surface. |
| 2..... | $C_8H_{17}-COO-(CH_2CH_2O)_{30}-SO_3Na$                  | 10                      |                                          |                                                                  |                                         |
|        |                                                          | 2                       |                                          |                                                                  |                                         |
|        |                                                          | 1                       | 43                                       | 88                                                               | 0.2-20 Do.                              |
| 3..... | Sulfuric acid ester of polyoxyethylene sorbitol stearate | 10                      |                                          |                                                                  |                                         |
|        |                                                          | 3                       |                                          |                                                                  |                                         |
|        |                                                          | 2                       | 43                                       | 84                                                               | 0.1-20 Do.                              |
| 4..... | $C_9H_{19}-C_6H_4-S-(CH_2CH_2O)_{30}-SO_3Na$             | 10                      |                                          |                                                                  |                                         |
|        |                                                          | 3                       |                                          |                                                                  |                                         |
|        |                                                          | 2                       | 43                                       | 85                                                               | 0.1-20 Do.                              |
| 5..... | $C_8H_{17}-CONH-(CH_2CH_2O)_{15}-SO_3Na$                 | 10                      |                                          |                                                                  |                                         |
|        |                                                          | 3                       |                                          |                                                                  |                                         |
|        |                                                          | 2                       | 42                                       | 84                                                               | 0.1-20 Do.                              |

From the data given in the above Tables 1 and 2, it will be understood that the zinc plating baths employing the three types of additives of the invention can produce substantially higher brilliance and surprisingly wider brilliance-imparting current density ranges as compared with those obtainable by the control prior art zinc plating baths.

For further better understanding of the present invention, several examples in which the present invention was successfully carried out will be given hereinbelow. However, it should be understood that the invention is not limited to the precise examples in any way.

## EXAMPLE 1

A zinc plating bath was prepared by adding 10 g/l of  $C_9H_{19}-COO-(CH_2CH_2O)_{20}SO_3Na$  as a sulfate compound of polyether, 3 g/l of 2-methyl-3-carboxyquinoline as a carboxylic acid compound of nitrogen-containing heterocyclic ring and 0.6 g/l of 5-chloro-2-acetylaphthylketone as an alkylaphthylketone compound to the fundamental composition comprising 120 g/l of zinc chloride and 190 g/l of ammonium chloride and a zinc plating operation was conducted using the bath under the conditions such as the temperature of 25°C, the pH of 5.0 and the current density of 5 A/dm<sup>2</sup> for 10 minutes. The obtained deposit metal had a high brilliance.

## EXAMPLE 2

A zinc plating bath was prepared by adding 8 g/l of  $C_9H_{19}-S-(CH_2CH_2O)_{30}SO_3Na$ , 4 g/l of 2-amino-3-carboxypyridine and 0.3 g/l of 6-ethyl-2-acetylaphthylketone to the fundamental composition comprising 90 g/l of zinc chloride, 200 g/l of ammonium chloride and 30 g/l of sodium gluconate and a zinc plating operation was conducted using the plating bath under the conditions as the temperature of 30°C, the pH of 5.0 and the current density of 2 A/dm<sup>2</sup> for 10 minutes. The obtained deposit metal had high covering power and brilliance.

## EXAMPLE 3

A zinc plating bath was prepared by adding 10 g/l of  $C_9H_{19}-OCH_2CH_2CH_2O-(CH_2CH_2O)_{50}SO_3Na$ , 3 g/l of nicotinic acid and 2.5 g/l of  $\beta$ -sulfo-2-acetylaphthylketone to the fundamental plating composition comprising 200 g/l of zinc sulfate, 30 g/l of ammonium chloride and 20 g/l of sodium salt of maleic acid and a zinc plating operation was conducted using the bath under the conditions such as the temperature of 25°C, the pH of 4.5 and the current density of 3 A/dm<sup>2</sup> for 10 minutes. The obtained deposit metal had a high brilliance.

## EXAMPLE 4

A zinc plating bath was prepared by adding 15 g/l of  $C_9H_{19}-C_6H_4-S-(CH_2CH_2O)_{20}SO_3Na$ , 5 g/l of 4-carboxyisoquinoline and 0.9 g/l of 5-methyl- $\beta$ -acetonaphthylketone to the fundamental composition comprising 40 g/l of zinc chloride and 230 g/l of ammonium chloride and a zinc plating operation was conducted using the bath under the conditions such as the temperature of 35°C, the pH adjusted to 7.2 with ammonia water and the current density of 2 A/dm<sup>2</sup> for 10 minutes. The obtained deposit metal had high brilliance and softness.

## EXAMPLE 5

A zinc plating bath was prepared by adding 5 g/l of  $H-O-(CH_2CH_2O)_{100}SO_3Na$ , 3 g/l of  $HS-(CH_2CH_2O)_{20}SO_3Na$  and 3 g/l of 4-carboxyisoquinoline and 0.3 g/l of 5-chloro- $\beta$ -acetyl- $\alpha$ -naphthylketone to the fundamental composition comprising 30 g/l of zinc chloride and 250 g/l of ammonium chloride and a zinc plating operation was conducted using the bath under the conditions such as the temperature of about 30°C, the pH of about 5.0 and the current density of 2 A/dm<sup>2</sup> for 10 minutes. The obtained deposit metal had a high brilliance.

While there have been described what are at present considered to be the preferred examples of this invention, it will be obvious to those skilled in the art that various changes and modifications may be made therein without departing from the invention, and it is aimed, therefore, in the appended appended claims to cover all such changes and modifications as fall within the true spirit and scope of the invention.

What is claimed is:

1. An aqueous cyanide-free zinc electroplating bath containing (a) a water soluble zinc salt selected from the group consisting of zinc chloride, zinc sulfate and zinc sulfamate, a water-soluble ammonium salt selected from the group consisting of ammonium chloride, ammonium sulfate and ammonium acetate, and optionally a hydroxycarboxylic acid; (b) from 0.1 to 30 gm/liter of at least one sulfate compound of the formula



wherein A is selected from the group consisting of hydrogen,  $C_nH_{2n+1}$  with n being an integer of 4 to 20, alkylphenyl, sorbitol, mannitol, alkylpolyamine, B is a member selected from the group consisting of  $-COO-$ ,  $-NH-$ ,  $-S-$ ,  $-O-$ ,  $-(OCH_2CH_2CH_2O)_{2-30}-$ , and  $-CONH-$ , and M is selected from the group consisting of hydrogen, ammonium, alkali metal, alkaline earth metal and zinc; (c) from 0.01 to 5.0 gm/liter of at least one alkylaphthylketone of the formula



wherein R<sub>1</sub> is selected from the group consisting of lower alkyl, phenyl, methylnaphthyl, styryl, nitrophenyl and aminophenyl and R<sub>2</sub> is selected from the group consisting of hydrogen, chlorine, bromine, lower alkyl, aryl, sulfo, amino, nitro, hydroxyl, carboxyl, and formyl; and (d) from 0.1 to 15 gm/liter of at least one nitrogen-containing heterocyclic ring compound having a carboxyl substituent of the formula



wherein



is a heterocyclic ring selected from the group consisting

of pyridine, quinoline and isoquinoline and R is selected from the group consisting of hydrogen, chlorine, lower alkyl, lower alkoxy, aryl, amino, nitro, hydroxyl, carboxyl, sulfo, sulfamoyl, hydroxylcarboxyl methylene, carboxy vinylene, carboxy phenyl, carboxy methyl, phenyl vinylene and mercapto.

2. The aqueous cyanide-free zinc electroplating bath of claim 1, in which said bath contains from 8 to 15 gm/liter of said sulfate compound.

3. The aqueous cyanide-free zinc electroplating bath

of claim 1, in which said bath contains from 0.3 to 2.5 gm/liter of said alkynaphthylketone.

4. The aqueous cyanide-free zinc electroplating bath of claim 1, in which said bath contains from 3 to 5 gm/liter of said heterocyclic ring compound.

5. The aqueous cyanide-free zinc electroplating bath of claim 1, in which the pH of said bath ranges from 3 to 10.

\* \* \* \* \*